

F. D. CARNEY & J. C. REED,  
HEAT TREATMENT OF RAILS,  
APPLICATION FILED AUG. 10, 1914.

1,188,148.

Patented June 20, 1916.



# UNITED STATES PATENT OFFICE.

FRANK D. CARNEY AND JOHN C. REED, OF STEELTON, PENNSYLVANIA.

## HEAT TREATMENT OF RAILS.

1,188,148.

Specification of Letters Patent. Patented June 20, 1916.

Application filed August 10, 1914. Serial No. 856,087.

To all whom it may concern:

Be it known that we, FRANK D. CARNEY and JOHN C. REED, citizens of the United States of America, residing at Steelton, in the county of Dauphin and State of Pennsylvania, have invented certain new and useful Improvements in Heat Treatment of Rails; and we do hereby declare the following to be a full, clear, and exact description of the invention, such as will enable others skilled in the art to which it appertains to make and use the same, reference being had to the accompanying drawings, and to letters or figures of reference marked thereon, which form a part of this specification.

Our invention relates to the improvement of the physical qualities of steel objects of approximately uniform cross sectional area of any desired length, such, for example, as 20 rolled shapes, and has for its object a novel method of treating such objects, to harden or toughen them uniformly throughout their whole length, or to both harden and toughen them, whereby the strength and resilience 25 may be increased to the maximum strength and resilience compatible with the composition of the steel may be secured, and utilized in the regular use of the steel object so treated.

30 While our invention is applicable to the treatment of steel objects of approximately uniform cross sectional area, whether produced by rolling, forging or casting, we have applied it more particularly to the improvement of steel railway rails, of maximum weight and length, such as used in tracks of heaviest traffic, and have found it practicable to secure remarkable uniformity in physical qualities, not only throughout the whole length of each, but also as compared with others of the same composition treated in like manner; thus, in securing an elastic limit of over 100,000 pounds per square inch, the variations of elastic 45 limit have not exceeded one-fifth of the variations of elastic limit found in similar material when treated in a furnace.

Having steel of a composition adapted to hardening and tempering whereby great increase of strength and durability was developed in objects conveniently heated and tempered, in view of the great need of more durable and reliable rails in the busier tracks of our important railways, the problem of 50 furnishing a tempered rail has become urgent, and was not easy to solve.

In the furnace treatments which we have tried, on standard rails of usual length, i. e., rails thirty-three feet long, the gas-fired furnace was forty-five feet long, including the ports. This length, and the doors for introducing the rails made it impossible to maintain constant temperatures throughout the entire length, and hence, obviously impossible to effect reliable tempering in any one rail, or uniformity in a 60 number of rails. Furthermore, the time required for the best possible furnace treatment, and the expense thereof, made it practically impossible to bring the cost low 65 enough to induce railways to consider adopting such rails. This, with the large proportion of imperfectly tempered rails, led us to seek for and devise a more reliable and cheaper method of tempering rails, capable 70 of producing a commercial product.

By our method of treating railway rails to harden and toughen them, generally speaking, the steel billet, bloom or ingot, having passed from the rolls where it is 75 shaped, is taken directly to the saws, then cambered, and immediately, while retaining as much as possible its initial heat, is dropped into a cooling fluid, or, to say, quenched. The quenched rail is then lifted 80 from the quenching tank, while having a temperature of about 300° C., is placed on insulated supports, and a heavy current of electricity passed through it from end to end to raise the temperature to a proper "temper 85 drawing" point, say about 450° C., or any other desired point above the quenched temperature. This operation requires only a few minutes, after which the rail passes onto the ordinary skids and receives the usual 90 handling to cold straighten, and to be drilled for splices. This method we have found to give a most satisfactory control over the physical properties of the steel. The tempering point, that is the temperature at 95 which the hardness of the quenched rail is reduced or drawn, can be controlled within a narrow limit, so that the properties of the steel in the rails may be made to conform to different requirements.

100 Another important advantage is that by varying the position and shape of the electrical contacts to the rails, we can produce a rail whose top, at the ends, will be harder than elsewhere, thereby enabling the rails 110 to resist the peening action of the car wheels when passing over the joints.

Another very valuable advantage is that by sending a current through the rails, the heating effect and drawing of the temper, is greatest in the interior, leaving the exterior harder than the interior, (just the opposite of the usual effect in furnace treatment) and this result is very advantageous.

Referring to the drawings, in which like parts are similarly designated, and in which we have diagrammatically shown a plant such as we have successfully used in tempering rails—Figure 1 is a diagrammatic plan view of a plant for tempering rails or bars of similar length; Fig. 2 is a side elevation, partly in section, of the quenching tank; Fig. 3 is an elevation showing one of the electric terminals from which current is supplied to the rail end, and the cooling device which may be used. Fig. 4 is a modification of Fig. 1, showing the use of a transformer in the electrical circuit; Fig. 5 is a further modification showing the use of a three phase current; Fig. 6 is a modification of Fig. 5, where pairs of rails are connected in three single phase sets.

A represents a roller mill, either of a two high reversing type, or the three high non-reversing type. The mill is driven by a motor 1, and its tables 2 and 3 are actuated from motors 4 and 5. The rails are delivered across the table 3 of the roller mill A to the saw-table B where they are sawed to proper length by the saws 6 and 7, after which they pass through a cambering machine, indicated at C, in order to have the proper curvature given to them so that the rails when cold will be straight or very nearly so.

The specific construction and operation of these machines is so well known in the art that a detailed description of their operation is deemed unnecessary.

D is a roller table, on which the cambered rails are received, and is in all respects similar to the roller table B. Cooperating with this table are two or more air cylinders 8 whose pistons carry pushers 9 arranged to push the rails *r* laterally off the table onto inclined guides 10 of a quenching tank E.

The lower part of the guides 10 is adjacent the lower end of a conveyer 11 which raises the rail from the water or other quenching fluid in the tank and deposits it on the temper drawing table F, and on supports 12 thereof of insulating material where the contact-shoes or cable terminals 13 are attached or otherwise placed in conductive relation to the ends of the rails. These shoes 13 are more clearly shown in Fig. 3, and are of copper or other suitable material, to which the electric cables conducting the current to be supplied to the rails are attached. These shoes have an upright portion 14 against which the end of the rail abuts. By varying the height of this abut-

ment 14, and thereby causing the current to enter and leave the ends of the rail through the foot, to a greater or less extent, rather than through the web or head, the current will take the path somewhat as shown by the dotted lines in Fig. 3, and thus not heat the ends of the top of the rail sufficiently to draw its temper at the ends of the rail head as much as elsewhere, and thus will leave this portion of the rail harder than elsewhere. The amount of heating of these ends of the top of the rail by convection will not be very great, since the time during which the current is passing through the rail is very short. However, if natural cooling in the air is not sufficient, or the hard area is to extend farther along the head toward the center of the rail, we place a water-cooled jacket 15 over the top of the rail as shown in Fig. 3, in order to chill that portion of the rail which we wish to be harder than the rest of the rail.

Direct current is supplied from a line L through a switch S and field rheostat 21 to a dynamo field 16, the armature P of which dynamo is driven by any suitable prime mover (not shown on the diagram). Alternating current will be generated in the armature P and will flow from P through the cable 17, contact or shot 13, rail *r*<sup>1</sup> contact 13<sup>a</sup>, cable 19, contact 13<sup>b</sup>, rail *r*<sup>2</sup> contact 13<sup>c</sup> ammeter A cable 18 and back to armature P. V is a voltmeter placed across the terminals of the rail. By adjusting the field rheostat 21 any desired current may be caused to flow through the rails. This we have found to be about 1000 amperes per square inch of cross section using a 25 cycle current and 50 volts pressure and two rails 100 lbs. per yard and 33 feet long in series. With a fixed current indicated on the ammeter A, the voltage indicated on the voltmeter V will increase as the temperature rises. If a pyrometer is placed on one of the rails and the voltage noted when the desired temperature is reached, the temperature of other rails, having the same sectional area and the same composition, can be determined directly from the voltmeter.

After the rails have been electrically reheated on the temper drawing table F they are moved onto the skids or cooling table 22. After cooling in the air, as usual with rails, they are cold straightened and drilled for splices.

In Fig. 4, we have shown a transformer T connected from a supply line L for alternating current through the switch S, the low tension side being connected to the terminals or shoes 13 and 13<sup>c</sup>. In this case the voltage V of the supply line is maintained constant, or nearly so, and the current shown on the ammeter A will drop as the temperature rises, and the desired temperature can be determined by consulting the ammeter,

the proper current having been previously determined for similar rails by the use of a pyrometer.

In Fig. 5 we show connections for three rails connected in a three phase circuit, and in Fig. 6 six rails connected as three single phase sets from a three phase circuit. We have found that it is desirable to use two rails, as shown in Fig. 4, three rails as shown in Fig. 5, or six rails as shown in Fig. 6, the last named being preferable when using a three phase source of supply of current, since it does not unbalance the system; all of which will be readily understood by those skilled in the use of electric current.

It is also desirable that two rails be treated simultaneously and side by side, since if only one rail is used, and the leads from the transformer connected to each end, it will cause a very much lower power-factor, which is objectionable, since this reduces the capacity of the electrical machinery and the lines. We have found that by placing the two rails side by side, but not in electrical contact, we more than double the power-factor over using one rail, so that a lower voltage is required to treat two rails in series than is required to treat one rail, using the same density of current; this is because of the induction between the two rails.

We find that with impedance seven times the resistance a 55% power-factor is obtainable. This is probably due to the fact that the rail has a high permeability at the temperatures at which we are working, and the very heavy electric current sets up a heavy magnetic field in and about the rails and causes secondary currents to flow within the rail, which assists the primary current in raising the temperature. There is also a considerable hysteresis loss within the rails, which also assists in heating them.

The time required to obtain the drawing temperature varies, of course, with the temperature of the rail at starting (after quenching) and the final desired temperature, and also with the amount and kind of current available. We find that using a current density of 1000 amperes per square inch of sectional area and from 50 to 75 volts pressure across two 33 foot rails connected in series, side by side, we can heat six pairs of rails, raising the temperature from 300° C. to 450° C. in six minutes, using a 25 cycle current. Direct current can be employed for this work, but it is objectionable, since a very much higher density of current would have to be employed, there being no secondary currents set up within the rails, and owing to the difficulty of transmitting such large currents any considerable distance without excessive losses, and the difficulties attending the providing of contacts for the larger currents required.

Of course the rails may be cold when treated, but it will take a longer time and more electrical energy to bring cold rails up to temper drawing temperature than hot rails, and in order to treat the rails economically we prefer to time the conveyor E so as to deliver the quenched rail to the tempering table at about 300° C.

It is, of course, obvious that other steel bars or shapes of approximately uniform cross-sectional areas, that from length or form are difficult to temper uniformly in a furnace, may be tempered by our method.

We claim—

1. The method of tempering previously hardened steel rails, which comprises passing an electric current through the rail sufficient to raise its temperature to the tempering point while maintaining the ends of the head of the rail cooler than the body of the rail.

2. The method of tempering steel rails proportioned for quenching, which comprises quenching the rail while retaining the heat incident to its manufacture in a quenching bath, withdrawing the rail from said bath while still hot but below the temper drawing point, and supplying a current of electricity longitudinally to the foot of the rail to raise its temperature to the temper drawing temperature.

3. The method of tempering steel rails, which comprises quenching the rail after rolling and while still hot from the quenching bath, passing an electric current through the rail to re-heat it to the temper drawing point, and then cooling the rail slowly.

4. The method of tempering rolled steel shapes, which comprises quenching the shape before becoming cool after its rolling operation to a temperature below the temper drawing point, and while still hot heating the shape up to the temper drawing point by passing an electric current therethrough from end to end.

5. The method of tempering steel rails, which comprises passing an electric current through the rail sufficient to heat it to its tempering point, while cooling the ends of the head of the rail.

6. The method of treating steel rails, which comprises quenching the rail to cool it below its tempering point, and then passing an electric current through the rail sufficient to heat it to its tempering point while cooling the ends of the head of the rail.

7. The method of treating steel rails, which comprises rolling the rail, cutting it to length, cambering it, quenching it to reduce its temperature to the neighborhood of 300° C., then passing an electric current through the rail to reheat it to the desired tempering point.

8. The method of tempering steel rails, which comprises passing an electric current

sufficient to heat the rails to the desired tempering point simultaneously through a plurality of rails that have been quenched below the tempering point but yet hot.

9. The method of tempering steel rails, which comprises passing an electric current sufficient to heat the rails to the desired tempering point simultaneously through a plurality of rails in inductive relation.

10. The method of tempering long, rigid steel shapes, which comprises heating a plurality of parallel shapes to their tempering point by passing a three-phase alternating electric current through them.

11. The method of tempering long, rigid steel shapes, which comprises heating a plurality of parallel shapes to their tempering point by passing a three-phase alternating electric current through them, said shapes being in inductive relation to one another.

12. The method of tempering long, rigid steel shapes, which comprises heating a plurality of such shapes that have been cooled below their tempering point, by heating them up to the tempering point desired by passing a three-phase alternating electric current longitudinally through pairs of such shapes arranged in single phase sets, the rails of each pair being in inductive relation.

13. The method of tempering steel rails, which comprises quenching the rail before it has lost the heat incident to its manufacture to cool it below its temper-drawing point, then passing a current of electricity through the rail, while still hot, to reheat it to the temper-drawing point, and allowing the rail to air-cool.

14. The method of tempering steel rails,

which comprises quenching the rails before they have lost the heat incident to their manufacture to cool them below their temper-drawing point, and then passing a current of electricity simultaneously through a plurality of such rails from end to end while still hot and in inductive relation to each other, to re-heat the rails to temper-drawing point.

15. The method of tempering steel rails, which comprises quenching the rails before they have lost the heat incident to their manufacture to cool them below their temper-drawing point, and then passing a current of electricity simultaneously through a plurality of such rails from end to end while still hot and in inductive relation to each other, to re-heat the rails to temper-drawing point and allowing the rails to air-cool.

16. The method of tempering steel rails, which comprises quenching the rails before they lose the heat incident to their manufacture to cool them below their temper-drawing point, then passing a current of electricity from end to end simultaneously through a plurality of the rails while still hot by supplying the current to the bases of the rails sufficient to re-heat them to their temper-drawing point, and then cooling the rails.

In testimony that we claim the foregoing as our invention, we have signed our names in presence of two subscribing witnesses.

FRANK D. CARNEY.  
JOHN C. REED.

Witnesses:

GEO. W. PARSONS,  
CHAS. R. HOLTON.